# EUROPEAN PATENT APPLICATION

(11) **EP 0 439 369 A1**
(43) Date of publication of application: **31.07.1991**
(21) Application number: 91300589.8
(22) Date of filing: 25.01.1991
(51) Int. Cl.: B41M 5/30, B41M 5/40

(54) **Heat-sensitive recording material**

(30) Priority: 25.01.1990 JP 15795/90
(71) Applicant: FUJI PHOTO FILM CO., LTD., Kanagawa (JP)
(72) Inventor: Mitsuo, Hirofumi, Fujinomiya-shi, Shizuoka (JP); Higashi, Shunsaku, Fujinomiya-shi, Shizuoka (JP)
(74) Representative: Moore, Anthony John (GB)

(57) **Abstract**

A heat-sensitive recording material comprises a support bearing at least a heat-sensitive recording layer comprising a binder, a color former and a developer. The heat-sensitive recording layer and/or a layer adjacent thereto contains at least one succinic compound.

The recording material has high sensitivity and is resistant to background fogging even after storage at high temperature.

## Description

This invention relates to a heat-sensitive recording material having high sensitivity and excellent capability to run through a facsimile machine, and which exhibits no substantial fogging when stored at high temperature.

Recording materials employing an electron donative dye precursor (referred to herein as a "color former") and an electron accepting compound (referred to herein as a "developer") are well known for use in such applications as pressure-sensitive recording paper, heat-sensitive recording paper, light-sensitive pressure-sensitive recording paper, electro conductive heat-sensitive recording paper and the like.

Such applications are disclosed in detail in, for example, British Patent 2,140,449, US Patent 4,480,052, US Patent 4,436,920, JP-B-60-23922 (the term "JP-B" as used herein means an "examined Japanese patent publication"), JP-A-57-179836 (the term "JP-A" as used herein means an "unexamined published Japanese patent application"), JP-A-60-123556 and JP-A-60-123557.

Because of the recently expanding use of heat-sensitive recording materials in various fields, there is a great demand for the improvement of the properties of these materials, especially for improvement in storage properties, namely, resistance to fogging on the background during storage for a long period of time, and/or at high temperature and the like.

Accordingly, an object of the present invention is to provide a heat-sensitive recording material having a high sensitivity and excellent capability to run through a facsimile machine, and which exhibits substantially no background fogging at high storage temperatures.

The above object is achieved by providing a heat-sensitive recording material comprising a support having thereon at least one layer, at least one layer of which is a heat-sensitive recording layer comprising a binder, a color former and a developer, the color-former reacts with the developer to form a color, wherein the heat-sensitive recording layer and/or a layer adjacent to the heat-sensitive color developing layer contains at least one compound selected from the group consisting of succinate-containing compounds represented by formulae (I), (II) and (III):
wherein R¹ and R², which may be the same or different, each represents hydrogen or an alkyl group having from 1 to 20 carbon atoms (which may be substituted); and X¹ and X², which may be the same or different, each represents hydrogen, an alkali metal, an ammonium or amine group (containing or not containing a substituent), which ammonium or amine group forms a salt with an acid group of the succinate.

The alkyl group represented by R¹ and R² preferably contains 1 to 8 carbon atoms, and is preferably a hydrogen atom or a lower alkyl group. Specific examples of the alkyl group represented by R¹ or R² include a methyl, ethyl, propyl, butyl and pentyl group.

Sodium and potassium are preferred as the alkali metal represented by X¹ or X², and triethanolamine and monoethanolamine are preferred as the amino group represented by X¹ or X².

The compound represented by formulae (I) to (III) for use in the present invention is preferably in the form of an alkali metal salt, more preferably in the form of a potassium salt. The compound represented by formulae (I) to (III) is added to the heat-sensitive recording layer and/or a layer adjacent to the heat sensitive recording layer in an amount of preferably from 5 to 200% by weight, more preferably from 10 to 100% by weight, based on the content of the color former.

An undercoat layer, a protecting layer and/or the like layer may be provided in the heat-sensitive recording material of the present invention and a layer adjacent to the heat-sensitive layer may contain at least one compound selected from succinic compounds represented by formulae (I), (II) and (III).

In the preparation of the heat-sensitive recording material of the present invention, a color former, a developer and a heat-fusible compound are disperseed in the presence of a water-soluble binder. The binder for use in the present invention is preferably selected from compounds which dissolve in water at 25°C in an amount of 5% by weight or higher. Useful examples of such compounds include polyvinyl alcohol, methyl cellulose, carboxymethyl cellulose, starch or a starch derivative including modified starch, gelatin, gum arabic, casein, a hydrolyzate of a styrene-maleic anhydride copolymer, a carboxy-modified polyvinyl alcohol, a polyacrylamide resin, a saponified product of a vinyl acetate-polyacrylic acid copolymer and the like. These binders may be used not only for the purpose of dispersion but also for the improvement of film strength for the latter purpose, a latex type synthetic polymer binder may be used together with the above described binders. Useful latex type binders include a copolymer of styrene and butadiene, a copolymer of vinyl acetate, a copolymer of acrylonitorile and butadiene, a copolymer of methyl acrylate and butadiene, polyvinylidene chloride and the like. These binders may also be applied to an undercoat layer.

The binder is generally used in an amount of from 5 to 20% by weight based on the total weight of solid content.

The color former for use in the present invention may be selected from triarylmethane compounds, diphenylmethane compounds, xanthene compounds, thiazine compounds, spiropyran compounds and the like. Useful examples of these compounds are disclosed, for example, in 1P-A-55-227253 which include: triarylmethane compounds such as 3,3′-bis(p-dimethyl-aminophenyl)-6-dimethylamino phthalide, 3,3′-bis(p-dimethylaminophenyl) phthalide, 3-(p-dimethylaminophenyl)-3-(1,3 dimethylindole-3-yl) phthalide and 3-(p-dimethyl-aminophenyl)-3-(2-methylindole-3-yl) phthalide; diphenylmethane compounds such as 4,4′-bis-dimethylamino-benzhydrin benzyl ether, N-halophenyl leucoauramine and N-2,4,5-trichlorophenyl leucoauramine; xanthene compounds such as Rhodamine B anilinolactam, Rhodamine-(p-nitrino) lactam, 2-(dibenzylamino) fluoran, 2-anilino-3-methyl-6-diethyl-aminofluoran, 2-anilino-3-methyl-6-dibutylaminofluoran, 2-anilino-3-methyl-6-N-ethyl-N-isoamylaminofluoran, 2-anilino-3-methyl-6-N-methyl-N-cyclohexylaminofluoran, 2-anilino-3-chloro-6-diethylaminofluoran, 2-anilino-3-methyl-6-N-ethyl-N-isobutylaminofluoran, 2-anilino-6-dibutylaminofluoran, 2-anilino-3-methyl-6-N-methyl-N-tetrahydrofurfurylaminofluoran, 2-anilino-3-methyl-6-piperidinoaminofluoran, 2-(o-chloro-anilino)-6-diethylaminofluoran and 2-(3,4-dichloroanilino)-6-diethylaminofluoran; thiazine compounds such as benzoyl Leucomethylene Blue and p-nitrobenzyl Leucomethylene Blue; spiropyran compounds such as 3-methyl-spiro-dinaphthopyran, 3-ethyl-spiro-dinaphthopyran , 3,3′-dichloro-spiro-dinaphthopyran, 3-benzylspiro-dinaphthopyran, 3-methyl-naphtho-(3-methoxy-banzo)-spiropyran and 3-propyl-spiro-dibenzopyran; and many other related compounds.

The color former is contained in the heat-sensitive recording layer in an amount of preferably from 0.1 to 2 g/m², more preferably from 0.2 to 1.0 g/m².

The developer for use in the present invention is preferably selected from phenolic compounds, salicylic acid derivatives and polyvalent metal salts thereof. Useful examples of these compounds include: phenolic compounds such as 2,2′-bis(4-hydroxyphenyl)propane, 4-t-butylphenol, 4-phenylphenol, 4-hydroxydiphenoxide, 1,1′-bis(3-chloro-4-hydroxyphenyl)cyclohexane, 1,1′-bis(4-hydroxyphenyl)cyclohexane, 1,1′-bis (3-chloro-4-hydroxyphenyl)-2-ethylbutane, 4,4′-sec-isooctylidenediphenol, 4,4′-sec-butylidenediphenol, 4-tert-octylphenol, 4-p-methylphenyl-phenol, 4,4′methylcyclohexylidene phenol, 4,4′-isopentylidene phenol and benzyl p-hydroxybenzoate; salicylic acid derivatives such as 4-pentadencyl salicylic acid, 3,5-di(α-methylbenzyl) salicylic acid, 3,5-di(ter-octyl)salicylic acid, 5-octadecyl salicylic acid, 5-α-(p-α-methylbenzyl-phenyl) ethyl salicylic acid, 3-α-methylbenzyl-5-ter-octyl salicylic acid, 5-tetradecyl salicylic acid, 4-hexyloxy salicylic acid, 4-cyclohexyloxy salicylic acid, 4-decyloxy salicylic acid, 4-dodecyloxy salicylic acid, 4-pentadecyloxy salicylic acid and 4-octadecyloxysalicylic acid; and zinc, aluminum, calcium, copper and lead salts of these salicylic compounds. Among the above described compounds and salts, phenolic compounds are particularly preferable because of their markedly high resistance to fogging on the background of the recording material.

The developer is contained in the heat-sensitive recording layer in an amount of from 50 to 800% by weight, more preferably from 100 to 500% by weight, based on the content of the color former. An amount of less than 50% by weight would cause insufficient color development and the addition of more than 800% by weight would not provide a proportionally greater effect.

For the purpose of improving thermal response of the heat-sensitive recording material of the present invention, a heat fusible compound may be included in the heat-sensitive recording layer. Useful examples of the heat fusible compound include benzyl p-benzyloxybenzoate, β-naphthyl-benzyl ether, stearic acid amide, stearylurea, p-benzyl-biphenyl, di(2-methylpehnoxy)ethane, di(2-methoxyphenoxy) ethan, β-naphthol-(p-methylbenzyl) ether, α-naphthylbenzyl ether, 1,4-butanediol-p-methylphenyl ether, 1,4-butanediol-p-isopropylphenyl ether, 1,4-butanediol-p-tert-octylphenyl ether, 1-phenoxy-2-(4-ethylphenoxy) ethane, 1-phenoxy-2-(4-chlorophenoxy) ethane, 1,4-butanediolphenyl ether, and diethyleneglycol-bis(4-methoxyphenyl) ether. The heat fusible compounds may be used alone or in combination thereof. For the purpose of obtaining sufficient thermal response, the heat fusible compound is used in an amount of from 10 to 200% by weight, more preferably from 20 to 150% by weight, based on the content of the developer.

Pigments for use in the present invention include calcium carbonate, barium sulfate, lithophone, agalmatolite, kaolin, silica, amorphous silica, aluminum hydroxide or the like.

As required, the heat-sensitive recording material of the present invention may include other commonly employed additives such as a metallic soap, a wax material, a surfactant, an antistatic agent, an ultraviolet ray absorption agent, an antifoaming agent, a conductive agent, a fluorescent dye and the like.

Useful metallic soaps include metal salts of higher fatty acids such as zinc stearate, calcium stearate and aluminum stearate.

Useful materials include a paraffin wax, a microcrystalline wax, a carnauba wax, methylolstearoamide, a polyethylene wax, a polystyrene wax, a fatty acid amide wax and the like either alone or in combination thereof.

Useful surfactants include an alkali metal salt of sulfosuccinic acid and a fluorine-containing surfactant.

The addition of an anti-decoloring agent to the heat-sensitive color developing layer is desirable for the purpose of preventing decoloring of image printed parts and thereby improving preservation of a formed image. Phenolic compounds, especially hindered phenol compounds, may be effective as the anti-decoloring agent. Useful examples of such compounds include 1,1,3-tris(2-methyl-4-hydroxy-tert-butylphenyl)-butane, 1,1,3-tris(2-ethyl-4-hydroxy-tert-butylphenyl)-butane, 1,1,3-tris(3,5-di-tert-butyl-4-hydroxyphenyl)butane, 1,1,3-tris(2-methyl-4-hydroxy-5-tert-butylphenyl)propane, 2,2′-methylene-bis(6-tert-butyl-4-methylphenol), 2,2′-methylene-bis(6-tert-butyl-4-ethylphenol), 4,4′-butylidene-bis(6-tert-butyl-3-methylphenol) and 4,4′-thio-bis(3-methyl-6-tert-butylphenol). The phenolic compound is preferably used in an amount of from 1 to 200% by weight, more preferably from 5 to 50% by weight, based on the content of the developer.

The above described ingredients are mixed together to form a coating solution, and the coating solution is then applied to a support. Useful supports include paper, synthetic paper or various bases, and an undercoat layer is preferably coated on the support prior to applying the coating solution for the recording layer to obtain a high smoothness. The heat-sensitive recording layer thus coated on a support is then dried and subjected to calendering treatment, etc., prior to practical use.

The present invention is illustrated below by reference to the following detailed Examples which should not be construed as limiting the present invention in any way.

### Example 1

### Preparation of undercoat paper:

A pigment dispersion was prepared by dispersing 80 g of a commercially available calcined kaolin (Ancylex 93, tradename, manufactured by Engelhard Corp.) in 160 g of a 0.5% aqueous solution of sodium hexametaphosphate using a homogenizer. The thus prepared pigment dispersion was mixed with 16 g of a styrene-butadiene latex (SN 307, tradename, manufactured by Sumitomo Nogatac Co., Ltd., solid content : 48%) and 24 g of a 10% aqueous solution of polyvinyl alcohol (PVA-117, tradename, manufactured by Kuraray Co., Ltd.) to obtain a coating liquid for use in providing an undercoat layer. Thereafter, the thus prepared coating liquid for an undercoat layer was applied onto the surface of a high quality paper having a weight of 50 g/m² in a coating weight 8 g/m². The thus treated paper was then dried to obtain an undercoat paper.

### Preparation and application of a coating solution for use in the formation of a heat-sensitive recording layer:

A mixture of 20 g of 3-dibutylamino-6-methyl-7-anilinofluoran and 100 g of a 5% aqueous solution of polyvinyl alcohol (PVA-105, tradename, manufactured by Kuraray Co., Ltd.) was treated in a ball mill for 24 to 48 hours to obtain a dispersion of particles having a mean particle size of 1.0 µm. Separately, a mixture of 40 g of bisphenol-A, 40 g of naphthylbenzyl ether and 400 g of a 10% aqueous solution of polyvinyl alcohol (PvA-105, tradename, manufactured by Kuraray Co., Ltd.) was treated in a ball mill for 24 to 48 hours to obtain a dispersion of particles having mean particle size of 1.0 µm. Also, using a homogenizer, a pigment dispersion was prepared by dispersing 80 g of calcium carbonate (Univer, tradename, manufactured by Shiraishi Kogyo Co., Ltd.) in 160 g of a 0.5% aqueous solution of sodium hexametaphosphate.

These three dispersions thus prepared were mixed together and the resulting mixture was further admixed with 50 g of 21% zinc stearate emulsion and 10 g of a compound represented by formula (I) wherein R¹ was hydrogen and X¹ and X² were potassium. A coating solution for use in the formation of a heat-sensitive recording layer thus prepared was then coated on the undercoated paper obtained above using a wire bar in such a manner that the density of the coated layer was 7 g/m² after drying. Thereafter, the thus coated undercoat paper was dried at 50°C in an oven to obtain a heat-sensitive recording material of the present invention.

### Example 2

A heat-sensitive recording material was prepared by repeating the procedure of Example 1, except that 10 g of the compound represented by formula (I) wherein R¹ was hydrogen and X¹ and X² were both potassium was replaced by 10 g of a compound represented by formula (II) wherein R¹ was hydrogen, R² was an n-pentyl group and X¹ and X² were potassium.

### Example 3

A heat-sensitive recording material was prepared by repeating the procedure of Example 1, except that 10 g of the compound represented by formula (I) wherein R¹ was hydrogen and X¹ and X² were both potassium was replaced by 10 g of a compound represented by formula (III) wherein R¹ and R² were n-butyl and X¹ and X² were potassium.

### Example 4

A heat-sensitive recording material was prepared by repeating the procedure of Example 1, except that 10 g of the compound represented by formula (I) in which R¹ was hydrogen and X¹ and X² were both potassium was replaced by 25 g of a commercially available 40% aqueous solution of alkenyl succinate (SizePine 5300, tradename, manufactured by Arakawa Kagaku Co., Ltd., which is a mixture of compounds of formulae (I) to (III) wherein R¹ and R² represented a mixture of alkyl groups having a total of 6 to 9 carbon atoms, and X¹ and X² were both potassium).

### Example 5

A heat-sensitive recording material was prepared by repeating the procedure of Example 3, except that the alkenyl succinate was removed from the heat-sensitive recording layer and 10 g of the same alkenyl potassium succinate as used in Example 3 was added to the coating liquid for the undercoat layer.

### Example 6

A heat-sensitive recording material was prepared by repeating the procedure of Example 3, except that the potassium salt of alkenyl succinate in the heat-sensitive recording layer was replaced by the triethanolamine salt.

### Example 7

A heat-sensitive recording material was prepared by repeating the procedure of Example 3, except that the addition amount of the potassium salt of the alkenyl succinate was reduced from 10 g to 1.6 g.

### Example 8

A heat-sensitive recording material was prepared by repeating the procedure of Example 3, except that the amount of the potassium salt of the alkenyl succinate was increased from 10 g to 24 g.

### Comparative Example 1

A heat-sensitive recording material was prepared by repeating the procedure of Example 1, except that the potassium salt of alkenyl succinate was not added to the coating liquid for the heat-sensitive recording layer.

### Evaluation of heat-sensitive recording paper:

Each of the thus prepared heat-sensitive recording materials was subjected to a surface treatment using a low pressure calender. Printing on the thus treated sheet of paper was carried out by using an experimental apparatus for heat-sensitive printing, equipped with a thermal head and a pressure roll (100 kg/cm²) attached directly to the thermal head (KLT-216-8MPD1, tradename, manufactured by Kyocera Corp.). Pressure rolling conditions of 24 V head voltage and 10 ms pulse cycle with the pulse width of 0.8, 1.0 and 1.2. Print density on the thus printed paper was measured using a Macbeth reflection density meter, model RD-918.

After storing the unrecorded heat-sensitive recording paper for 3 days in a thermo- and hygro-stat under a constant temperature of 60°C and a constant moisture of 30% RH, fogging value on the background of the recording material was measured using the same Macbeth reflection density meter, model RD-918.

Results of the evaluation are shown in Table 1. It is clearly seen that the heat-sensitive recording material of the present invention exhibits substantially no fogging of the background even after storage at a high temperature.

Thus, the present invention provides a heat-sensitive recording material having a high sensitivity and an excellent facsimile running capacity and which exhibits substantially no fogging of the background during storage at high temperature

## Claims

1. A heat-sensitive recording material comprising a support having provided thereon at least a heat-sensitive recording layer comprising a binder, a color former and a developer, the color former being capable of reacting with the developer to form color, characterised in that the heat-sensitive recording layer and/or a layer adjacent to the heat-sensitive recording layer contains at least one compound selected from succinic compounds represented by the following general formulae (I) to (III): wherein R¹ and R², which may be the same or different, each represent a hydrogen atom or an alkyl group having from 1 to 20 carbon atoms; and X¹ and X², which may be the same or different, each represent a hydrogen atom, an alkali metal atom, or an ammonium or amino group, which ammonium or amino group forms a salt with an acid group of the succinic compound.

2. A recording material as claimed in claim 1, in which the one or more succinic compounds represented by formulae (I) to (III) are contained in the heat-sensitive recording layer.

3. A recording material as claimed in claim 1 or 2, in which the one or more succinic compounds represented by formulae (I) to (III) are contained in an undercoat layer provided between the support and the heat-sensitive recording layer.

4. A recording material as claimed in claim 1, 2 or 3, in which at least one succinic compound represented by formulae (I) to (III) is in the form of a potassium salt.

5. A recording material as claimed in any preceding claim, in which the one or more succinic compounds represented by formulae (I) to (III) are present in an amount of from 5 to 200% by weight based on the content of the color former.

6. A recording material as-claimed in any preceding claim, in which the developer is a phenolic compound.

7. A recording material as claimed in any preceding claim, in which the developer is contained in the heat-sensitive recording layer in an amount of from 50 to 800% by weight based on the content of the color former.

8. A recording material as claimed in any preceding claim, in which the color developing layer further contains a heat fusible compound in an amount of from 10 to 200% by weight based on the content of the developer.
